

## UNITED STATES PATENT OFFICE.

REGINALD HILL MONK, OF MONTREAL, QUEBEC, CANADA.

## METHOD OF OBTAINING TITANIUM OXIDE.

No Drawing.

Application filed July 7, 1926. Serial No. 121,058.

This invention relates to the treatment of minerals and products thereof containing titanium, such as ilmenite, rutile after the elimination of impurities and a large portion 5 of the iron content, and particularly titanium concentrates such as are obtained by the process described in U. S. Patent No. 1,543,250, 16th June 1925.

The object of my invention is to convert 10 such refractory compounds of titanium into a water soluble compound, or compounds. This I propose to do by the use of a mixture of sulphuric acid with an alkali metal sulphate, at a temperature lower than that at 15 which a true fusion of the alkali acid sulphate takes place. Under such conditions and at this temperature there is very little loss of the free acid present, which is an aid when dissolving the resultant mass in water.

20 The further object is to produce an aqueous solution of titanium compounds especially adapted for the preparation of pure titanium oxide and hydroxides thereof.

25 A further object is the production of titanium oxide especially suited for use as a white pigment. The solution obtained by my invention possesses new and desirable qualities whereby is assured the precipitation of titanium compounds entirely free from impurities, such as iron, which causes discoloration 30 of the final product.

The solution obtained is novel in itself, as hydrolysis may be carried out at a very low 35 temperature. Providing the iron present has previously been reduced to the ferrous state, the compound of titanium obtained on hydrolysis is entirely free from impurities. The temperature employed is so low that the ferrous iron is not oxidized during the process, and no hydrolysis of iron salts takes place.

40 I am aware that various patents have been granted for the sulphating of titanium ores and the products thereof, but these processes are invariably carried out at relatively high 45 temperatures at which fusion occurs.

The melt obtained from the employment of such substances as concentrated sulphuric acid or sodium bisulphate, or combinations of these two, does not produce a large 50 portion of water soluble sulphates if a high temperature is used.

This is more particularly shown in the case of the above mentioned titanium concentrates obtained by the process described 55 in Letters Patent No. 1,543,250.

When rutile, or other refractory minerals and products thereof, have been subjected to a temperature around 1000° C. the process of direct treatment with concentrated sulphuric acid decomposes only a small percentage of 60 the titanium present, and fusion of the residue at comparatively high temperatures with salts of alkali metals does not result in the production of a large percentage of titanium 65 compounds soluble in water.

This invention relates to a process in which one continuous operation only is carried out at a temperature much lower than is required when an alkali metal salt is used alone. Furthermore, no other addition of acid is required 70 in order to bring the titanium into aqueous solution. The process differs from that using sulphuric acid only, as in addition to sulphuric acid large quantities of sodium sulphate are employed. The acid alone reacts 75 with only a small percentage of the titanium present, whereas the use of the sodium acid sulphate and sulphuric acid mixture, as described, effects a complete decomposition of 80 the titanium oxides.

The process differs from fusion with acid alkali metal sulphates alone, since in addition to such sulphates, sulphuric acid is also employed, and during the treatment the optimum temperature leading to the formation 85 of soluble titanium compound is employed. This temperature is about 160° C. below that at which the sodium acid sulphate fuses, which is 300° C.

Furthermore, practically no acid is driven 90 off, and the titanium is entirely soluble in water without any addition of acid. At the low temperature employed no alkali titanites are formed.

In order to fully describe my invention I 95 state the following example:

From a titanium concentrate, obtained by the process described in Patent No. 1,543,250, containing 19.93% total iron, 7% metallic iron, and 54.62%  $TiO_2$ , I take 400 grams, mix 100 this with 600 grams of  $NaHSO_4$ , and 840 grams  $H_2SO_4$ , 66.43%. This mixture is now heated to 120° C., being agitated the meanwhile. The mass is kept below 140° C. for three hours. When it shows a tendency to solidify it is transferred on to a flat tray, and the temperature raised to 260° C. for a short time, until a solid cake is formed. The cake is allowed to cool, disintegrated, and lixiviated with cold water.

Resulting solution contains:

|                                       | Grams<br>per litre. |
|---------------------------------------|---------------------|
| Fe.....                               | 31.9                |
| TiO <sub>2</sub> .....                | 71.2                |
| 5 So <sub>3</sub> (total).....        | 331                 |
| Na <sub>2</sub> SO <sub>4</sub> ..... | 99                  |

From this solution titanic oxide precipitates even in the cold, if it is allowed to stand. 10 I prefer to hasten the hydrolysis by bringing the temperature up to 75° C. in the course of about 1½ hours, the iron having been previously reduced to the ferrous state. Titanic oxide now precipitates slowly, free from 15 impurities, and as the acid in the solution increases, being liberated by the hydrolysis of the titanium compound. I raise the temperature gradually, and finally bring it up to 95° C., or thereabouts, for the last 20 to 20 30 minutes. In this manner a pure compound of titanium is precipitated, and all the iron is kept in solution.

What I claim is:—

1. The method of converting refractory 25 compounds of titanium after the elimination of impurities and a large portion of the iron content into water soluble sulphates, comprising mixing the comminuted compound with an alkali-metal sulphate and an acid 30 solvent, heating the mixture at a temperature from 120° to 300° C., until a solid cake is formed, cooling and crushing the cake.

2. The method of converting refractory 35 compounds of titanium after the elimination of impurities and a large portion of the iron content into water soluble sulphates, comprising mixing the comminuted compound with an alkali-metal sulphate and an acid 40 solvent, heating the mixture at first below 140° C. transferring to a tray and raising the temperature to about 260° C. until a solid cake is formed, cooling and crushing the cake and lixiviating with cold water.

3. The method of obtaining titanium oxide 45 from concentrates containing titanium and iron which comprises, mixing the comminuted material with an alkali-metal sulphate and an acid solvent, heating the mixture at a temperature from 120° to 300° C. until a 50 solid cake is formed, cooling and crushing the cake and lixiviating with cold water, and precipitating the titanium oxide from the solution.

4. The method of obtaining titanium oxide 55 from concentrates containing titanium and iron which comprises mixing the com-

minuted material with an alkali-metal sulphate and an acid solvent, heating the mixture at a temperature from 120° to 300° C. until a solid cake is formed, cooling and crushing the cake, lixiviating with cold water and hydrolyzing the solution at a low temperature.

5. The method of obtaining titanium oxide 60 from concentrates containing titanium and iron which comprises, mixing the comminuted substance with an alkali-metal sulphate and an acid solvent, heating the mixture below 140° C. transferring the mass to a tray and raising the temperature to about 70 260° C. until a solid cake is formed, cooling and crushing the cake, lixiviating with cold water and precipitating the titanium oxide from the solution.

6. The method of obtaining titanium oxide 75 from concentrates containing titanium and iron which comprises, mixing the comminuted substance with an alkali-metal sulphate and an acid solvent, heating the mixture below 140° C. transferring the mass to 80 a tray and raising the temperature to about 260° C. until a solid cake is formed, cooling and crushing the cake, lixiviating with cold water, reducing the iron to the ferrous state and precipitating the titanium oxide from 85 the solution.

7. The method of obtaining titanium oxide 90 from concentrates containing titanium and iron which comprises, mixing the comminuted material with approximately one and one half times by weight of an alkali-metal sulphate and double the weight of sulphuric acid, heating the mixture to below 140° C. until it begins to solidify, heating on a flat 95 tray up to 260° C. till a solid cake is formed, cooling and crushing the cake and then lixiviating with cold water and precipitating the titanium oxide from the solution.

8. The method of obtaining titanium oxide 100 from concentrates containing titanium and iron which comprises, mixing the comminuted material with approximately one and a half times by weight of an alkali-metal sulphate and double the weight of sulphuric acid, heating the mixture to below 140° C. until it begins to solidify, heating on a flat 105 tray up to 260° C. till a solid cake is formed, cooling and crushing the cake and then lixiviating with cold water and hydrolyzing the solution at not over 75° C. and gradually to 110 about 95° C.

REGINALD HILL MONK.